

# United States Patent Office

3,788,955

Patented Jan. 29, 1974

1

3,788,955

## ENCAPSULATION

Nelson A. Crites and Glenn R. Schaer, Columbus, Ohio, assignors to Battelle Development Corporation, Columbus, Ohio

No Drawing. Continuation-in-part of abandoned application Ser. No. 117,059, Feb. 19, 1971. This application Oct. 7, 1971, Ser. No. 187,560

Int. Cl. B01i 13/02; C23b 5/56, 17/00

U.S. Cl. 204—25

26 Claims

## ABSTRACT OF THE DISCLOSURE

Encapsulation of liquids with metal. A core liquid is dispersed in a carrier liquid in which it is essentially insoluble (one of the liquids being aqueous), in a container whose surface is phobic to the core liquid. Metallizing and reducing compounds are added. Nucleating metal is deposited at the interface between the liquids by introducing a surfactant-type metal-organic compound of the hydrophobic-hydrophilic type having a more readily oxidizable metal ion than the metal of the metallizing agent, so that molecules of the surfactant align themselves at the interface and present their metal ions to the aqueous liquid to nucleate deposition of metallizing ions. In one embodiment, the metallizing materials are disposed to deposit a noble metal at the interface, and the resulting noble-metal-coated capsules are subsequently over-coated with one or more layers of a non-noble metal by electrodeposition.

## RELATED APPLICATION

This application is a continuation-in-part of our co-pending U.S. patent application Ser. No. 117,059, filed Feb. 19, 1971, now abandoned.

## BACKGROUND

There is a growing demand for encapsulated liquids for applications such as carbon-paper-less copy paper, cigarette filter water release, etc. Additionally, there are now uses for encapsulated liquids such as the electrically conductive capsules for use in the indicating coatings of co-pending patent application Ser. No. 11,418, filed Feb. 16, 1970, now abandoned, entitled "Indicating Coating." Said application has been replaced by a continuation filed Sept. 25, 1972, Ser. No. 291,690.

Such demands are currently met by processes such as those described in U.S. Pat. No. 2,800,458, B. K. Green, wherein a nonpolar liquid to be encapsulated is dispersed in a polar carrier liquid in which it is insoluble. The coating material consists of a protein or gelatinous material such as gelatin or a vegetable gum which is added to the carrier liquid and caused to coagulate through the phenomenon of syneresis by adjustment of solution pH and/or temperature or other suitable means entrapping the nonpolar (i.e., oily) liquid to effect microencapsulation.

Other well known prior art means for encapsulating liquids include the substantial reverse of the above-described procedure. In this process an aqueous solution is dispersed in a nonaqueous-nonpolar solvent liquid containing dissolved hydrophobic polymerized material. A nonaqueous nonpolar liquid in which the polymerized material is insoluble is added to the dispersion to cause the polymerized material to precipitate out of solution and form capsule walls around the aqueous phase. This method is taught by U.S. Pat. 3,173,878.

Various other means for encapsulation include coating a solid material and replacing the solid with a liquid by leaching as taught in U.S. Pat. 3,460,972 and spray coating fluidized frozen liquids as taught in U.S. Pat. 3,202,533.

2

One of the most important requirements for encapsulated liquids relates to the integrity of the capsule wall. Nearly all of the above procedures provide capsule walls of organic materials that are inherently porous. Thus, the "shelf life" or period during which the capsules will effectively hold or retain the liquid core is limited.

## THE INVENTION

We have now discovered a method whereby liquid cores may be encapsulated with metals. A continuous metal case exhibits substantially no porosity and, consequently, our method provides liquid-filled capsules with greater "shelf life" than any of the presently known encapsulation procedures.

We disperse the core liquid in, or form an emulsion of, this liquid with a carrier liquid in which the core liquid is insoluble or immiscible. We then add a metallizing material such as a silvering solution that is used to coat glass in the manufacture of mirrors and an appropriate reducing agent to affect appropriate reduction of the metallizing compounds and make metal ions available for deposition.

As in the case of glass metallizing or silvering the interface between the liquid (liquid we are encapsulating) and the carrier liquid must be activated or deposition must be nucleated before capsule walls (silvering) will occur. In the silvering of glass, catalysts such as tin chloride are adsorbed onto the glass surface prior to treatment. The tin ions being readily oxidizable are displaced

by reducing silver ions at random sites on the glass surface nucleating the deposition of silver ions. In the present instance, however, the usual catalytic metal compounds such as tin chloride obviously cannot be applied to the interface between the core liquid and the carrier liquid.

Thus, catalytic nucleation of metallizing or the deposition of metal ions in the conventional sense is not possible.

Where the liquid to be encapsulated is immiscible in water and the carrier liquid is aqueous, we have found that such catalytic action may be effected through the use of surfactants that consist of polar metal-organic compounds. These compounds, like detergents, have a hydrophilic end (the organic end) and a hydrophobic end (the metal-containing end). The metal ion located at the hydrophilic end of the molecule in the present instance consists of a metal that is more readily oxidized than the metal of the metallizing compound. Thus, this surfactant functions as a catalyst in initiating deposition at the interface between the core liquid and the carrier liquid since the molecule will align itself at the interface with its hydrophobic end toward the liquid to be encapsulated and its hydrophilic end toward the carrier, exposing the readily oxidizable metal ion to replacement with a reduced metallizing ion to initiate deposition.

The catalytic surfactant of the present invention may be any metal-organic compound (or molecule) having a hydrophilic part or end that includes a metal that is more readily oxidizable than the metal to be deposited (or reduced) and a hydrophobic part or end that will seek out the nonaqueous emulsion at the emulsion interface presumably to escape the water and thus expose the metal to oxidation. The metal-organic compound must possess some solubility in water although this may be slight since only a small amount of catalytic or nucleating action is generally required to effect encapsulation. For example, any metal salt of an alkyl acid may be employed providing such salts meets the above-described parameters. Also, some aryl salts such as stannous benzoate or tartrate may be employed in appropriate circumstances. Further, alkyl or aryl metal chelates may be used in some instances.

The most available metal-organic compounds or molecules for use in conjunction with the method of the present invention are the metal salts of the fatty acids

particularly those ranging in carbon from about 4 carbon atoms to 18 carbon atoms. Such compounds that contain less than 4 carbon atoms would tend to dissociate in the usual ammoniacal metallizing solution while the limited solubility of those exceeding about 18 carbon atoms would be very slight. Such compounds may be saturated or unsaturated since this parameter does not enter into the function of the addition.

We have had particular success in using stannous compounds (i.e., stannous octoate  $\text{Sn}(\text{O}_2\text{CC}_7\text{H}_{15})_2$ ) as our catalytic surfactant, however, as set forth above, any metal salt may be employed so long as the metal is more readily oxidizable than the metal of the metallizing salt.

We have found that the catalytic surfactant may be added either to the core liquid or to the carrier liquid (or to both). Where making the addition to the core liquid, it is, of course, most convenient to make the addition prior to the formation of the emulsion. Where the addition is to be made to the carrier liquid, it can be made either before or after the formation of the emulsion or the addition of the metallizing and metallizing-reducing additions.

The metal-organic hydrophilic-hydrophobic surfactant utilized in conjunction with the method of the present invention must also be compatible with the nonpolar liquid or liquid to be encapsulated. By compatible, we mean at least partially soluble and the liquid to be encapsulated cannot be of a type to interfere with proper alignment at the emulsion liquid-liquid interface to nucleate metallizing. For example, if the liquid to be encapsulated has as great as or greater affinity for the hydrophilic portion of the surfactant as the carrier liquid, it will not align itself at the interface in the desired manner. We have found that highly halogenated organic liquids such as carbon tetrachloride and chloroform, though immiscible in water, are generally incompatible with the usual hydrophobic-hydrophilic metal organic surfactant.

Metallizing compositions or solutions are not confined to silvering compositions or solutions although the greatest utilization of this coating technique is in coating glass to provide mirrors.

Most silvering solutions are comprised in part of an ammoniacal solution of silver nitrate (usually containing some alkali metal hydroxide) plus a reducing solution which functions to convert the ammoniacal silver to the metallic form.

Other well-known metallizing compositions or solutions include copper coating baths which are very similar to silvering solutions. For example, one such solution, is disclosed in U.S. Pat. 2,939,804, Schossberger et al., which consists of 35 g./l. of copper sulfate



and 173 g./l. of sodium hydroxide ( $\text{NaOH}$ ).

Still further commonly used metallizing solutions include gold, platinum, palladium, cobalt, and nickel compounds (for nickel compounds see U.S. Pat. No. 3,420,680, Galla).

The reducing agent may be any material capable of reducing the metal compound of the metallizing solution to render anions or positive metal ions available for cationic deposition at the interface between the core liquid and the carrier liquid. Common reducing agents for silvering solutions are formaldehyde, Rochelle salts (sodium potassium tartrate), sugar, and hydrazine. The recommended reducing agent for the aforementioned copperizing solution is Fehling's solution.

The noble metals such as silver, gold, platinum, and palladium deposit on the interface surface more readily than metals such as copper, nickel, and cobalt. The reason for this is that the known reducing agents and catalytic surfactants are far more efficient in reducing these metals to their elemental or metallic state than metals

such as nickel and cobalt. However, it is economically highly desirable to effect capsule walls of metals such as nickel and cobalt rather than the noble metals. An effective way of accomplishing the desired result is to effect a small or minor coating of a noble metal (i.e., Au, Ag, Pt, and Pd) through the use of an appropriate metallizing solution, reducing agent, and catalytic surfactant and then over-coating the noble metal coating with the desired metal coat. Since the capsules possess a coat of noble metal, the noble metal will itself nucleate deposition of metal from other metallizing solutions such as solutions for the deposit of nickel, cobalt, and copper. Such a noble metal coat may be so thin as to be imperceptible and may be noncontinuous but will serve to nucleate metal deposition from other metallizing materials.

Metallizing compounds and reducing agents may be added to the emulsion with the addition of the catalytic surfactant in minor properties for the limited deposition of a noble metal and, subsequently, metallizing compounds and reducing agents may be added to the same emulsion in greater proportions to effect a complete encapsulation with a non-noble metal (for example, Ni, Cu, or Co). Any number of encapsulating metal layers may be effected in this manner.

Alternately, capsules thinly coated with a noble metal in the manner described above may be over-coated with one or more second coatings by conventional electroplating. For example, we have electroplated copper onto the surface of capsules of silver coated silicone by floating the capsules on a copper sulfate bath and contacting the capsules with a horizontal cathode plate.

For some applications, such as for use in the indicating coating of U.S. patent application Ser. No. 11,418, now abandoned, the core liquid may be a liquid capable of carrying an electric current. For example, a conductive liquid may consist of a solution of ammonium chloride and glycerine. Such a solution may be dispersed in an aqueous solution and metallize coated in the manner described above. Where the liquid one proposes to encapsulate is not electrically conductive, it may be rendered electrically conductive by incorporating a dispersion of carbon particles therein. For example, we have rendered ethylene glycol electrically conductive by making 2 percent, by weight, additions of borax and 5 percent, by weight, SC Carbon (milled).

The particulate carbon addition may, of course, come from any essentially elemental carbon source. For example fine lampblack is an excellent source of powder for this application, however, granular or flake graphite can also be used. The particle size of the carbon can be critical and the carbon particles can be any size that will provide adequate electrical conductivity. Preferably, however, the carbon will be at least fine enough to pass through a 50-mesh screen.

Where the liquid to be encapsulated is not electrically conductive, the carbon may be dispersed therein by means of mechanical agitation. The liquid then becomes a conductive liquid which is in turn dispersed in the carrier liquid. Appropriate surfactants can be added to the electroconductive liquid to maintain the carbon dispersion and appropriate surfactants such as emulsifiers may be added for the carrier liquid to maintain the emulsion or dispersion of the conductomer liquid in the carrier during coating.

We have had surprising success in both maintaining the emulsion of the electrically conductive liquid in the carrier liquid and in preventing the carbon particles from separating from the conductive liquid by adding a single wetting agent (FC-95 Surfactnt, manufactured by 3M Company or J. P. Stevens 915, both fluorocarbon detergents) to the carrier liquid that will perform this function.

Especially good results are obtained when the emulsion comprises also a wetting agent that enhances the stability of the emulsion. The wetting agent typically comprises a

surfactant that is at least slightly soluble in both the core liquid and the carrier liquid, such as sodium lauryl sulfate, a fluorocarbon detergent, or an alkyl phenyl polyethylene glycol ether. It is also preferred that the materials be held in a container whose surface is phobic to the core liquid, and the emulsion may beneficially comprise also a wetting agent that increases the phobic char-

5 allowed to form liquid-liquid interfaces. A silver nitrate silvering solution was mixed with the water phase of each test. A silvering solution reducing agent (Rochelle Salts), when used, was also mixed with the water phase. Varying surfactants (where used) were added to the water-immiscible liquid. The results are set forth in the following table:

TABLE I

| Test number | Water-immiscible liquid | Surfactant            | Silver nitrate solution | Rochelle salts | Results           |
|-------------|-------------------------|-----------------------|-------------------------|----------------|-------------------|
| 1           | Mineral oil             | None                  | Yes                     | Yes            | No silvering.     |
| 2           | do                      | 502 <sup>1</sup>      | Yes                     | Yes            | Silvering.        |
| 3           | do                      | T-9 <sup>2</sup>      | Yes                     | Yes            | Do.               |
| 4           | Dibutyl phthalate       | T-9                   | Yes                     | Yes            | Do.               |
| 5           | do                      | 502                   | Yes                     | Yes            | Do.               |
| 6           | Carbon tetrachloride    | T-9                   | Yes                     | Yes            | No silvering.     |
| 7           | Chloroform              | T-9                   | Yes                     | Yes            | Do.               |
| 8           | Platinum chloride       | None                  | Yes                     | Yes            | Do.               |
| 9           | Silicone oil            | 502                   | Yes                     | Yes            | Silvering.        |
| 10          | do                      | 502                   | Yes                     | No             | No silvering.     |
| 11          | do                      | Tributyl tin chloride | Yes                     | Yes            | Silvering.        |
| 12          | do                      | None                  | Yes                     | Yes            | No silvering.     |
| 13          | do                      | Tributyl tin chloride | Yes                     | No             | Do.               |
| 14          | do                      | Butyl titanate        | Yes                     | Yes            | Silvering.        |
| 15          | do                      | do                    | Yes                     | No             | No silvering.     |
| 16          | do                      | Benzylaldehyde        | Yes                     | Yes            | Do.               |
| 17          | do                      | Butyraldehyde         | Yes                     | Yes            | Do.               |
| 18          | do                      | Benzylaldehyde        | Yes                     | No             | Do.               |
| 19          | do                      | Butyraldehyde         | Yes                     | No             | Do.               |
| 20          | do                      | Tributyl tin chloride | Yes                     | Butyraldehyde  | Slight silvering. |
| 21          | do                      | do                    | Yes                     | Benzaldehyde   | Do.               |

<sup>1</sup> A silicone rubber catalyst, manufactured by Dow Corning Company, the active ingredient of which consists of stannous octoate.

<sup>2</sup> A silicone rubber catalyst, manufactured by M. & T Chemicals, Inc., the active ingredient of which consists of stannous octoate.

acter of the container surface. This wetting agent typically comprises a surfactant that is soluble in the carrier liquid, such as alcohol sulfates, sodium salts, and alkylaryl sulfonates where the carried liquid is aqueous, and such as fluorocarbon and fluorophosphate detergents where the carrier liquid is nonaqueous. Where the core liquid comprises water, the container surface preferably comprises polyethylene, polytetrafluoroethylene polystyrene, or other polymerized organic plastic, and the carrier liquid preferably consists essentially of a substantially water-insoluble oil, typically an organic oil such as toluene or mineral oil. The metallizing materials typically comprise essentially silver nitrate; ammonia; magnesium sulfate; and, as a reducing compound, Rochelle salts; and the metal-organic surfactant compound typically consists essentially of stannous octoate. In certain uses such as in marking or covering markings, the diameters of at least about 90 percent of the capsules should be about 50 to 150 microns, with an average diameter of about 75 to 125 microns.

#### EXAMPLES

(1) 115 cc. water was placed in a 250 ml. beaker. (2) 15 cc. of 1%, by weight, FC-95 surfactant (3M Company) was added. (3) About 2 cc. of silicone oil containing carbon particles was added. (4) A stirrer was used to disperse the oil droplets in the water. The surfactant prevented the droplets from coalescing and the carbon from separating from the oil. (5) Three drops of Dow Corning Corporation 502 silicone rubber catalyst was added. The active ingredient of this catalyst is tin octoate. (6) Silvering solution and reducing solution concentrates were added to form a silver-mirror coating solution. (7) Stirring was continued for 30 minutes and the silver-coated droplets of oil were washed by decanting several times with water containing the surfactant. (8) Several of the silver-coated droplets were copper electroplated by floating them on an acid copper sulfate bath and contacting them with a horizontal cathode plate. After plating for a short time, the metal-coated spheres sank to the bottom of the tank.

A series of tests were conducted to determine the operability of various materials when used in conjunction with the method of the present invention. In each of these tests water immiscible liquids were mixed with water and

35 From the above data, it is obvious that to effect metal encapsulation in accordance with the method of the present invention one must employ a metal-organic surfactant of a metal that is more readily oxidizable than the metallizing (silvering) metal. The surfactant must be of the hydrophilic-hydrophobic type and must be compatible with the nonpolar liquid.

#### FURTHER EXAMPLES

##### (A) Encapsulating oil droplets with silver

40 (1) 250 ml. of a solution of a wetting agent such as 350 mg. of surfactant FC-95 (3M Company) per liter in distilled water, is prepared. This is a preferred, but optional, step which provides the wetting agent recited in some of the claims. (2) 4 ml. of light mineral oil are dispersed in the solution with vigorous stirring for about 5 minutes. (3) ten drops (about 350 mg.) of a stannous-octoate catalyst such as T-9 (M&T Chemicals Corporation) are added to the oil-water dispersion with reduced stirring for about 2 minutes. This step provides the metal-organic surfactant compound recited in the claims. (4) 45 Sixty ml. of an equivolume mix of silver-reducer concentrates are added to the oil-catalyst-water dispersion (about 1.3 g. of Ag/310 ml.) with mild stirring for about 20 minutes. The first four steps may be carried out in any other convenient order, or substantially simultaneously, if desired. (5) Stirring is stopped and the dispersion is allowed to settle. Because the coating is very thin, the silver-coated droplets produced appear light gray-black to the naked eye. (6) About 125 ml. of the dispersion containing coated oil drops are decanted into 175 ml. of a solution similar to that of Step (1) (about 300 mg. FC-95 per liter). This is is another preferred, but optional, step for providing a wetting agent. (7) A second 60 ml. mix of the silver-reducer concentrates is added to the decanted dispersion mix, to complete the silvering reaction after standing for at least about an hour. To increase the thickness of the silver wall, this step may be repeated. (8) Most of the capsules now have a metallic silver appearance. (9) The capsules are rinsed, collected on filter papers, and air dried. (10) Where stronger coatings are desired, the capsules are further coated with copper as in the other examples or in any other convenient manner.

## (B) Encapsulating water-containing droplets

(1) To a 500 ml. capacity polyethylene bottle the following reagents are added:

- (a) About 50 ml. toluene. (Mineral oil can be used in place of part or all of the toluene.)
- (b) About 0.1 gram stannous octoate (M&T's T-9).
- (c) About 0.1 gram surfactant FC-95 (3M). This is an optional material, providing the wetting agent recited in some of the claims.
- (d) About 0.5 ml. of a silvering solution. A typical silvering solution contains about 0.25 ml. of  $\text{AgNO}_3$  (70 g./l.) with  $\text{NH}_4\text{OH}$  (about 80 ml./l.), and about 0.25 ml. 425 g./l. Rochelle salts with 30 g./l.  $\text{MgSO}_4 \cdot 7\text{H}_2\text{O}$ . It may be conveniently injected by hypodermic needle and syringe to produce small droplets.

(2) The mixture is allowed to stand for about 2 to 24 hours.

Tests with Example (B) show that for best yields the surface of the container should be phobic to the liquid to be encapsulated. When water is the core liquid a hydrophobic material such as polyethylene, polytetrafluoroethylene, polystyrene, or other polymerized organic plastic is satisfactory. Glass and metal are not.

The following additional steps are also recommended: (3) The resulting silver coated spherical capsules are poured onto an electroless copper plating solution comprising about 15 g./l. copper nitrate ( $\text{CuNO}_3 \cdot 3\text{H}_2\text{O}$ ), 10 g./l. sodium bicarbonate ( $\text{NaHCO}_3$ ), 30 g./l. Rochelle salts, and 20 g./l. sodium hydroxide ( $\text{NaOH}$ ), but without the usual formaldehyde reducer. (4) The mixture is allowed to stand until the toluene has evaporated. This typically requires about one to twenty-four hours. (5) About 100 ml. per liter of formaldehyde (37-38% HCHO) are added. (6) The mixture is allowed to stand for about one to two hours. (7) The copper plated spheres are removed from the plating solution.

What is claimed is:

1. The process of forming capsules having a liquid core and a metal case comprising:
  - (a) forming an emulsion of the core liquid in a carrier liquid, one said liquid being aqueous and the other being substantially water-immiscible and the emulsion being held in a container whose surface is phobic to the core liquid;
  - (b) introducing metallizing materials, including a reducing compound, into said emulsion; and
  - (c) nucleating metal deposition from said metallizing materials at the interface between said core liquid and said carrier liquid by introducing into said emulsion a metal-organic surfactant compound that is at least partially soluble in both said core liquid and said carrier liquid and which is compatible with said water-immiscible liquid, the metal containing part of said surfactant being philic to said aqueous liquid and the nonmetal part being phobic to said aqueous liquid so that the molecules of said surfactant will align themselves at the interface of said core and carrier liquids with the philic parts directed to the aqueous liquid, the metal of said surfactant being more readily oxidizable than the metal of said metallizing compound in the environment of the emulsion so that at least some of the metal ions of the surfactant will reduce metal ions of said metallizing compound to a metallic state to nucleate metallizing of the interface between said core liquid and said carrier liquid;
  - (d) wherein said metallizing materials provide at least one metal selected from the group consisting of Ag, Cu, Au, Pt, Pd, Co, and Ni and said surfactant consists essentially of butyl titanate or of a stannous salt of a fatty acid having from about 4 to 18 carbon atoms.

2. The method of claim 1 wherein said carrier liquid consists essentially of water and said core liquid consists essentially of a substantially water-insoluble oil.

3. The process of forming capsules having a liquid core and a metal case comprising:

- (a) forming an emulsion of the core liquid consisting essentially of a substantially water-insoluble oil in a carrier liquid consisting essentially of water, said liquids being substantially immiscible in one another;
- (b) introducing metallizing materials, including a reducing compound into said emulsion, said metallizing materials providing an ammoniacal solution of a silver compound and a reducing material that functions to convert the silver to the metallic form; and
- (c) nucleating metal deposit from said metallizing materials at the interface between said core liquid and said carrier liquid by introducing into said emulsion a metal-organic surfactant compound consisting essentially of a stannous salt of a fatty acid having from about 4 to 18 carbon atoms that is at least partially soluble in both said core liquid and said carrier liquid and which is compatible with said core liquid, the metal containing part of said surfactant being philic to said carrier liquid and the nonmetal part being phobic to said carrier liquid so that the molecules of said surfactant will align themselves at the interface of said core and carrier liquids with the philic parts directed to the carrier liquid, the metal of said surfactant being more readily oxidizable than the metal of said metallizing compound in the environment of the emulsion solution so that at least some of the metal ions of the surfactant will reduce metal ions of said metallizing compound to a metallic state to nucleate metallizing of the interface between said core liquid and said carrier liquid.

4. The method of claim 3 wherein said core liquid consists essentially of a silicone oil.

5. The method of claim 4 wherein said silver compound consists of silver nitrate.

6. The method of claim 4 wherein said silicone oil is provided with a dispersion of carbon particles therein that are disposed to render said oil electrically conductive.

7. The method of claim 2 wherein a wetting agent is added to said emulsion to maintain said emulsion.

8. The method of claim 6 wherein a wetting agent is added to said emulsion to maintain said emulsion and to maintain the dispersion of said carbon particles.

9. The process of claim 1 wherein said metallizing materials are disposed to deposit a noble metal at said interface and said noble-metal-coated capsules are subsequently over-coated with one or more layers of a non-noble metal.

10. The process of claim 9 wherein said noble metal is at least one metal selected from the group consisting of Ag, Au, Pt, and Pd and said non-noble metal is at least one metal selected from the group consisting of Cu, Ni, and Co.

11. The process of claim 10 wherein the noble-metal-coated capsules are coated with the non-noble metals by exposure to one or more metallizing solutions of the non-noble metals so that the noble-metal coatings act as catalysts for deposition of one or more of the non-noble metals.

12. The process of claim 10 wherein the noble-metal-coated capsules are coated with one or more of the non-noble metals by electrodeposition in a plating solution of the non-noble metal.

13. The method of claim 1 wherein said surfactant is added to said core liquid prior to forming said emulsion.

14. A process as in claim 1, wherein the emulsion comprises also a wetting agent that enhances the stability of the emulsion.

15. A process as in claim 1, wherein the emulsion comprises also a wetting agent that increases the phobic character of the container surface.

16. A process as in claim 1, wherein the core liquid comprises water and the container surface comprises polyethylene, polytetrafluoroethylene, polystyrene, or other polymerized organic plastic.

17. A process as in claim 1, wherein the core liquid consists essentially of water and the carrier liquid consists essentially of a substantially water-insoluble oil.

18. A process as in claim 17, wherein the carrier liquid consists essentially of toluene.

19. A process as in claim 17, wherein the carrier liquid consists essentially of mineral oil.

20. A process as in claim 17, wherein the metallizing materials comprise essentially silver nitrate; ammonia; magnesium sulfate; and, as a reducing compound, Rochelle salts.

21. A process as in claim 20, wherein the metal-organic surfactant compound consists essentially of stannous octoate.

22. A process as in claim 14, wherein the wetting agent comprises essentially a surfactant that is at least slightly soluble in both the core liquid and the carrier liquid.

23. A process as in claim 15, wherein the wetting agent comprises essentially a surfactant that is soluble in the carrier liquid.

24. A process as in claim 1, wherein the metal-organic surfactant compound consists essentially of stannous octoate.

25. A process as in claim 1, wherein the average diameter of the capsules is about 75 to 125 microns.

26. A process as in claim 1, wherein the diameters of at least about 90 percent of the capsules are about 50 to 150 microns.

#### References Cited

#### UNITED STATES PATENTS

|           |         |               |       |             |
|-----------|---------|---------------|-------|-------------|
| 2,757,104 | 7/1956  | Howes         | ----- | 117—160 R X |
| 3,390,026 | 6/1968  | Cerych et al. | ---   | 117—160 R X |
| 3,406,119 | 10/1968 | Kosar et al.  | ----- | 252—316     |
| 3,468,662 | 9/1969  | McCune, Jr.   | ---   | 252—313 R X |
| 3,503,783 | 3/1970  | Evans         | ----- | 252—316 X   |

RICHARD D. LOVERING, Primary Examiner

U.S. CL. X.R.

117—71 R, 100 A, 100 B, 160 R, 217, 227; 204—38 B; 252—316; 264—4

UNITED STATES PATENT OFFICE  
CERTIFICATE OF CORRECTION

Patent No. 3,788,995 Dated January 29, 1974

Inventor(s) Frederick A. Stahly and Steward H. Merrill

It is certified that error appears in the above-identified patent and that said Letters Patent are hereby corrected as shown below:

Column 5, line 73, "Zince" should read --Zinc--;

Column 6, line 64, "Alkll" should read --Alkyl--;

Column 7, line 27, "prsent" should read --present--;

Column 8, line 56, "electristatic" should read  
--electrostatic--;

Column 14, line 53, the word --high-- should be inserted  
after the word having;

Column 17, line 18, the part of the sentence reading  
"dissolving g." should read --dissolving 1 g.--;

Column 17, line 33, after the word developer, insert ---.---;

Column 17, line 47, "5" should read --15--;

Column 17, lines 57 and 58, after the words methacrylate-  
co-, insert --lauryl methacrylate-dimethylaminoethyl  
methacrylate-co- --;

Column 17, line 65, the period "." should be deleted  
after the word, Isopar G;

Column 23, line 59, "sulfoalkl" should read --sulfoalkyl--;

Column 25, line 60, "VII" should read --VIII--.

Signed and sealed this 17th day of September 1974.

(SEAL)

Attest:

McCOY M. GIBSON JR.  
Attesting Officer

C. MARSHALL DANN  
Commissioner of Patents